# EUROPEAN PATENT SPECIFICATION

(11) **EP 1 008 676 B1**
(45) Date of publication and mention of the grant of the patent: **26.05.2004**
(21) Application number: 99830766.4
(22) Date of filing: 09.12.1999
(51) Int. Cl.: C23G 3/02, C23G 1/08

(54) **Accelerated steel strip pickling process and device for carrying out the process**
Beschleunigtes Verfahren zum Beizen von Stahlband und Vorrichtung dafür
Procédé accéléré de décapage de bandes en acier et dispositif pour exécuter le procédé

(30) Priority: 10.12.1998 IT RM980761
(43) Date of publication of application: 14.06.2000
(73) Proprietor: CENTRO SVILUPPO MATERIALI S.p.A., 00129 Roma (IT)
(72) Inventor: Dulcetti, Alessandro, c/o C. Sviluppo Mat. S.p.A., 00129 Roma (IT); Giannetti, Armando, c/o C. Sviluppo Mat. S.p.A., 00129 Roma (IT)
(74) Representative: Leone, Mario

(56) References cited:
- EP-A- 0 513 753
- WO-A-88/01657
- DE-A- 4 240 572
- GB-A- 2 031 036
- US-A- 1 780 594
- US-A- 5 282 485
- US-A- 5 879 465
- PATENT ABSTRACTS OF JAPAN vol. 009, no. 112 (C-281), 16 May 1985 (1985-05-16) & JP 60 005888 A (MITSUBISHI JUKOGYO KK), 12 January 1985 (1985-01-12)
- PATENT ABSTRACTS OF JAPAN vol. 013, no. 442 (C-641), 3 October 1989 (1989-10-03) & JP 01 168883 A (SUMITOMO CHEM CO LTD), 4 July 1989 (1989-07-04)

## Description

The present invention relates to the continuous pickling in a non-oxidizing acid bath of hot-rolled strips of magnetic and stainless ferritic steels.

As it is known, often annealed and non-annealed magnetic steels and some annealed stainless steels have surface oxides, as scale and/or internal oxidation, highly adherent and with low reaction rates inside the conventional non-oxidizing pickling baths. Oxides possibly remaining on the surface after the pickling can cause serious inconveniences in the downstream treatments, and can interfere with the magnetic characteristics and the surface finishes of the two types of steel considered.

At present, the state of the art substantially provides three possible interventions for obtaining pickled surfaces that are completely clean of oxides. The first intervention comprises the use of non-oxidizing pickling baths with very lengthy immersion times. The second possible intervention comprises the addition of hydrofluoric acid to the pickling bath. Lastly, the third type of intervention comprises the use of oxidizing baths with the entailed cost-effectiveness and environmental impact drawbacks. However, none of those extremely aggressive methods can preserve the non-oxidized matrix of the underlying steel. Moreover, the adoption of the first type of intervention (anyhow including lengthy treatment times that entail negative repercussions on productivity) is hindered by the occurrence of inconveniences due to operational problems, whereas the adoption of the second and of the third type of intervention are hindered by cost-effectiveness and environmental protection reasons.

Therefore, notwithstanding research efforts, in the specific field object still remains for a pickling process that is simple, fast, cost-effective and of a negligible environmental impact.

The present invention permits to satisfy this object, further showing other advantages that will be apparent hereinafter.

Following the above, the present invention is related to a process for the continuous pickling, in a non-oxidizing acid bath, of hot-rolled steel strips, characterised in that the strip to be pickled is subject to the pickling action of the bath additioned with a pickling catalyst, under turbulent conditions, the pickling catalyst being at least one organic compound including at least one thiolic group. Satisfactory results were obtained with an organic compound comprising at least one thiolic group selected from a list comprising thioglycolic acid, its ammonium salt, and combinations thereof.

The concentration of the organic compound comprising a thiolic group inside the pickling bath is comprised in the range 0.005-0.01 moles/litre.

A further object of the present invention is a device apt to carry out the aforedescribed process.

This device is characterised in that it comprises the following components in combination:
- a closed storage tank containing a pickling bath, additioned with a pickling catalyst consisting of at least one organic compound comprising at least one thiolic group;
- at least one cell, located above the free surface of the pickling bath, inside which the strip to be pickled, possibly guided by supporting rolls, travels horizontally;
- immersed nozzles, provided above and below the strip, located and shaped so as to feed under pressure the pickling bath to the cell, to create a directional flow of the pickling bath itself that generates the required turbulent conditions;
- means for drawing the pickling bath from the tank and delivering it to the nozzles; and
- means for recirculating the pickling bath from the cell to the tank.

The means for drawing the pickling bath from the tank and delivering it to the nozzles can be a pumping circuit.

The means for recirculating the pickling bath from the cell to the tank can be a slit-shaped overflow inside the cell from which the bath cascades into the tank.

The cell body can be monolithic and integral with the storage tank, or it can be made of two overlapped portions, the lower thereof being integral with the tank, whereas the upper thereof is integral with the cover of the tank, thus being movable.

The most important technical effect yielded by the invention is that of accelerating the mass transfer at the interface with the surface to be pickled, and in performing a mechanic action to ease the detachment of oxide residues therefrom.

The present invention can be applied to the conventional pickling baths inclusive of non-oxidizing acids, thereby increasing the pickling capacity thereof.

The invention can also be applied with reasonable costs to the extant immersion pickling lines in order to improve/accelerate the performances thereof.

The accelerating effect is most evident for oriented and nonoriented, hot-rolled, annealed or non annealed magnetic steels, and the annealed ferritic stainless steels (AISI 400).

The deriving combined effect permits to obtain for the magnetic steels, the quantity of dissolved material being equal, clean surfaces with 30 to 60% shortened immersion times, even in presence of internally oxidized zones that usually are not easily pickled. Alternatively, the final performance being equal, the temperature and/or the acidity of the pickling bath can be decreased. The yielded surfaces are clean of oxides, and smoother than the ones yielded by the non-additioned pickling systems.

Likewise results are obtained with the ferritic stainless steels (series 400) for which the pickling rate can be doubled.

So far, only a general description of the present invention has been provided. A more detailed description of some specific embodiments thereof will hereinafter be provided with reference to the figures and examples, aimed at making better understood the objects, characteristics, advantages and operational modes thereof.
Figure 1 is a schematic side view of an embodiment of the turbulence tank according to the present invention.
Figure 2 is a schematic front view of the embodiment of the turbulence tank according to the invention depicted in figure 1.
Figure 3 shows the weight loss values function of the pickling time, and the linear interpolation for a nonoriented magnetic steel (Si= 3%, Al= 0.5%), pickled in a pickling solution including hydrochloric acid at 80°C, with and without the application of the present invention.
Figure 4 shows the weight loss values function of the pickling time, and the linear interpolation for an AISI 430 stainless steel, pickled in a pickling solution including sulphuric acid at 80°C, with and without the application of the present invention.

### Example 1

A 2-mm thick nonoriented magnetic steel (Si= 3.0%, Al= 0.5%) in a hot-rolled annealed state was immersed for increasing times in a pickling solution including 140 g/l HCl, 90 g/l FeCl2, at 80°C, under static conditions. Then the test was repeated using a turbulence cell according to the present invention, in presence of 0.006 moles/l accelerating additive.

With reference to figures 1 and 2, the closed storage tank containing the catalyst-additioned pickling bath is indicated with 1, the three cells in a sequence, having the top portion thereof integral to the movable cover 7 of the tank are indicated with 2, positioned above the free surface of the bath, inside which the strip to be pickled, guided by supporting rolls 3, travels horizontally. The reference number 4 indicates submersed nozzles, located above and below the strip, positioned and shaped so as to feed under pressure the pickling bath to the cell, thereby creating a directional flow of the pickling solution itself that generates the required turbulent conditions.

The reference number 5 indicates the pumping circuit that draws the solution from the storage tank and delivers it to the nozzle batteries.

The pickling solution exits by the overflow from each cell through the slit 6 and cascades into the tank 1.

The concentration of the accelerating additive (thioglycolic acid) in the pickling solution is 0.005 moles/l.

The results reported in figure 3 show that, weight losses being equal, the application of the present invention permits a 30 to 60% reduction in the immersion time, or that, immersion times being equal, an approximate 30% increase of the weight loss is obtained.

### Example 2

An AISI 430 stainless steel, hot-rolled and annealed, was immersed for increasing times in a pickling solution including 200 g/l H2SO4, 80 g/l FeSO4, at 80°C, under static conditions. Then the test was repeated using the turbulence device according to the present invention adopted in example 1, in presence of 0.005 moles/l accelerating additive.

The results reported in figure 4 show that, weight losses being equal, the application of the present invention permits a 65% reduction in the immersion time, or that, immersion times being equal, a 165 to 220% increase in weight loss is obtained.

## Claims

1. A process for the continuous pickling, in a non-oxidizing acid bath, of hot-rolled steel strips, **characterised in that** the strip to be pickled is subject to the action of the pickling bath, additioned with a pickling catalyst, under turbulent conditions, the pickling catalyst being at least one organic compound comprising at least one thiolic group.

2. The process for the continuous pickling of hot-rolled steel strips in a non-oxidizing acid bath according to claim 1, wherein the organic compound comprising at least one thiolic group is selected from a list comprising thioglycolic acid, its ammonium salt and combinations thereof.

3. The process for the continuous pickling of hot-rolled steel strips in a non-oxidizing acid bath according to any one of the preceding claims, wherein the catalyst concentration inside the pickling bath is comprised in the range 0.005-0.01 moles/litre.

4. A device apt to carry out the process according to claims 1 to 3, **characterised in that** it comprises the following components in combination:
- a closed storage tank (1) containing a pickling bath, additioned with a pickling catalyst consisting of at least one organic compound comprising at least one thiolic group;
- at least one cell (2), positioned above the surface of the pickling bath, inside which the strip to be pickled, possibly guided by supporting rolls (3), travels horizontally.
- immersed nozzles (4), located above and below the strip, positioned and shaped so as to feed under pressure the pickling bath to the cell (2), in order to create a directional flow of the pickling bath itself that generates the required turbulent conditions;
- means (5) for drawing the pickling bath from the tank (1) and delivering it to the nozzles (4); and
- means (6) for recirculating the pickling bath from the cell (2) to the tank (1).

5. The device according to claim 4, wherein the means (5) for drawing the pickling bath from the tank (1) and delivering it to the nozzle (4) is a pumping circuit.

6. The device according to any one of the claims 4 and 5, wherein the means (6) for recirculating the pickling bath from the cell (2) to the tank (1) is a slit-shaped overflow, inside the cell, wherefrom the pickling bath cascades into the tank (1).

7. The device according to any one of the preceding claims, wherein the body of the cell is monolithic and integral with the storage tank (1).

8. The device according to any one of the claims 4 to 6, wherein the body of the cell is made of two overlapped portions, the lower thereof is integral with the tank (1), whereas the upper thereof is integral with the cover (7) of the tank, and therefore is movable.

## Patentansprüche

1. Verfahren zum kontinuierlichen Beizen von warm gewalzten Stahlbändern in einem nichtoxidierenden Säurebad, **dadurch gekennzeichnet, dass** das zu beizende Band der Wirkung des Beizbades, dem ein Beizkatalysator zugesetzt wird, unter turbulenten Bedingungen ausgesetzt wird, wobei der Beizkatalysator wenigstens eine organische Verbindung ist, die wenigstens eine Thiolgruppe umfasst.

2. Verfahren zum kontinuierlichen Beizen von warm gewalzten Stahlbändern in einem nichtoxidierenden Säurebad nach Anspruch 1, wobei die organische Verbindung, die wenigstens eine Thiolgruppe umfasst, aus einer Liste ausgewählt wird, die Thioglycolsäure, deren Ammoniumsalz und Kombinationen derselben umfasst.

3. Verfahren zum kontinuierlichen Beizen von warm gewalzten Stahlbändern in einem nichtoxidierenden Säurebad nach einem der vorhergehenden Ansprüche, wobei die Katalysatorkonzentration innerhalb des Beizbades in dem Bereich von 0,005-0,01 Mol/Liter liegt.

4. Vorrichtung zum Ausführen des Verfahrens nach den Ansprüchen 1 bis 3, **dadurch gekennzeichnet, dass** sie folgende Komponenten in Kombination umfasst:
- einen geschlossenen Lagertank (1), der ein Beizbad enthält, welchem ein Beizkatalysator zugesetzt ist, der aus wenigstens einer organischen Verbindung besteht, die wenigstens eine Thiolgruppe umfasst;
- wenigstens eine Zelle (2), die oberhalb der Oberfläche des Beizbades angeordnet ist und innerhalb welcher sich das zu beizende Band horizontal bewegt, gegebenenfalls geführt durch Stützwalzen (3),
- eingetauchte Düsen (4), die oberhalb und unterhalb des Bandes angeordnet und so positioniert und geformt sind, dass sie das Beizbad der Zelle (2) unter Druck zuführen, um eine gerichtete Strömung des Beizbades selbst zu erzeugen, die die verlangten turbulenten Bedingungen erzeugt;
- eine Einrichtung (5) zum Abziehen des Beizbades aus dem Tank (1) und zum Fördem desselben zu den Düsen (4); und
- eine Einrichtung (6) zum Zurückleiten des Beizbades aus der Zelle (2) in den Tank (1).

5. Vorrichtung nach Anspruch 4, wobei die Einrichtung (5) zum Abziehen des Beizbades aus dem Tank (1) und zum Fördern desselben zu der Düse (4) ein Pumpkreis ist.

6. Vorrichtung nach Anspruch 4 oder 5, wobei die Einrichtung (6) zum Zurückleiten des Beizbades aus der Zelle (2) in den Tank (1) ein schlitzförmiger Überlauf innerhalb der Zelle ist, von dem aus das Beizbad in Kaskaden in den Tank (1) gelangt.

7. Vorrichtung nach einem der vorhergehenden Ansprüche, wobei der Körper der Zelle monolithisch und integral mit dem Lagertank (1) ausgebildet ist.

8. Vorrichtung nach einem der Ansprüche 4 bis 6, wobei der Körper der Zelle aus zwei überlappten Teilen besteht, von denen der untere mit dem Tank (1) integral ausgebildet ist, wohingegen der obere integral mit dem Deckel (7) des Tanks ausgebildet und daher beweglich ist.

## Revendications

1. Procédé pour le décapage continu, dans un bain d'acide non-oxydant, de bandes d'acier laminées à chaud, **caractérisé en ce que** la bande devant être décapée est soumise à l'action du bain de décapage, enrichi d'un catalyseur de décapage, sous des conditions turbulentes, le catalyseur de décapage étant au moins un composé organique comportant au moins un groupe thiolique.

2. Procédé pour le décapage continu de bandes d'acier laminées à chaud dans un bain d'acide non-oxydant selon la revendication 1, dans lequel le composé organique comportant au moins un groupe thiolique est sélectionné à partir d'une liste comportant acide thioglycolique, son sel d'ammonium et des combinaisons de ceux-ci.

3. Procédé pour le décapage continu de bandes d'acier laminées à chaud dans un bain d'acide non-oxydant selon l'une quelconque des revendications précédentes, dans lequel la concentration de catalyseur à l'intérieur du bain de décapage est située dans la plage allant de 0,005 à 0,01 mole/litre.

4. Dispositif apte à mettre en oeuvre le procédé selon l'une quelconque des revendications 1 à 3, **caractérisé en ce qu'**il comporte les composants suivants en combinaison :
- un réservoir de stockage fermé (1) comportant un bain de décapage, enrichi d'un catalyseur de décapage constitué d'au moins un composé organique comportant au moins un groupe thiolique,
- au moins une cellule (2), positionnée au-dessus de la surface du bain de décapage, à l'intérieur de laquelle la bande devant être décapée, guidée de manière possible par des rouleaux de support (3), se déplace horizontalement,
- des buses immergées (4), situées au-dessus et au dessous de la bande, positionnées et mises en forme de manière à alimenter sous pression le bain de décapage vers la cellule (2), pour créer un écoulement directionnel du bain de décapage lui même qui génère les conditions turbulentes nécessaires,
- des moyens (5) pour extraire le bain de décapage à partir du réservoir (1) et l'acheminer vers les buses (4), et
- des moyens (6) pour remettre en circulation le bain de décapage à partir de la cellule (2) vers le réservoir (1).

5. Dispositif selon la revendication 4, dans lequel les moyens (5) pour extraire le bain de décapage à partir du réservoir (1) et l'acheminer vers les buses (4) sont constitués d'un circuit de pompage.

6. Dispositif selon la revendication 4 ou 5, dans lequel les moyens (6) pour remettre en circulation le bain de décapage à partir de la cellule (2) vers le réservoir (1) sont constitués d'un trop-plein en forme de fentes, à l'intérieur de la cellule, à partir duquel le bain de décapage tombe en cascade dans le réservoir (1).

7. Dispositif selon l'une quelconque des revendications précédentes, dans lequel le corps de la cellule est monolithique, et est en un seul bloc avec le réservoir de stockage (1).

8. Dispositif selon l'une quelconque des revendications 4 à 6, dans lequel le corps de la cellule est constitué de deux parties en chevauchement, la partie inférieure étant en un seul bloc avec le réservoir (1), tandis que la partie supérieure est en un seul bloc avec le couvercle (7) du réservoir, et est par conséquent mobile.
